

# UNITED STATES PATENT OFFICE.

NINEVEH R. BONNER AND IRA L. BURLINGAME, OF PANA, ILLINOIS.

## PAINT COMPOUND.

SPECIFICATION forming part of Letters Patent No. 409,904, dated August 27, 1889.

Application filed April 25, 1889. Serial No. 308,549. (No specimens.)

*To all whom it may concern:*

Be it known that we, NINEVEH R. BONNER and IRA L. BURLINGAME, of Pana, in the county of Christian and State of Illinois, have invented a new and Improved Paint Compound, of which the following is a full, clear, and exact description.

This invention consists in a paint or paint compound which is more particularly designed for use upon roofs, whether made of tin, iron, wood, or other material.

The composition consists of the following ingredients, combined in or about the proportions stated, viz: mortar-cement, preferably hydraulic, one-half bushel; yellow ocher, eight pounds; Venetian red, eight pounds; rosin, eight pounds; sulphur, six pounds; alum, six pounds; burnt umber, six pounds; lamp-black, six pounds; Spanish asbestos, six pounds; asphaltum, six pounds. These several ingredients are thoroughly mixed together, and to every four gallons of such mixture we add half a gallon of liquid japan and mix the whole with twelve gallons of coal-tar.

In applying this paint compound to a roof the same is heated till it boils, and then put on with an ordinary whitewash or other suitable brush.

Said paint or paint compound will not only be water-proof, but will also serve to make the roof fire-proof so far as falling sparks and cinders on it are concerned. It will stop a leak if no larger than an ordinary nail-hole, and will not scale, crack, peel, blister, or fall off. Atmospheric changes from hot to cold, or vice versa, will not affect it, and it will not eat into the metal or wood surface to which it is applied, and will be found exceedingly durable.

Having thus described our invention, what we claim as new, and desire to secure by Letters Patent, is—

The herein - described paint composition, consisting of mortar-cement, yellow ocher, Venetian red, rosin, sulphur, alum, burnt umber, lamp-black, asbestos, asphaltum, liquid japan, and coal-tar, in or about the proportions specified.

NINEVEH R. BONNER.  
IRA L. BURLINGAME.

Witnesses:

J. W. SMITH,  
I. N. WEAVER.